

## UNITED STATES PATENT OFFICE

2,196,009

HARD ALLOYS AND METHOD FOR  
PRODUCING THE SAME

Walther Dawihl, Berlin - Kohlhasenbruck, and  
Karl Schröter, Berlin, Germany, assignors to  
General Electric Company, a corporation of  
New York

No Drawing. Application December 6, 1938, Se-  
rial No. 244,222. In Germany January 11,  
1938

8 Claims. (Cl. 106—1)

Our invention relates to hard alloys and to a method for producing the same.

In the production of hard alloys used in the cutting, that is, chip-removing and in the non-cutting shaping treatment carbides are used, as a rule, in particular carbides of metals of high melting point. Tool bodies of such carbides are produced frequently by heating the carbides or carbide mixtures up to melting and allowing them to solidify, under circumstances in suitable molds. The shaped bodies thus obtained show a comparatively coarse-crystalline texture which prejudice their use for many purposes. Consequently, shaped bodies have been prepared from powdered carbides at normal temperature by pressing which pressed bodies subsequently are strengthened merely by sintering. In order to obtain with this method sufficient hardness of the shaped bodies, the sintering frequently has been raised up to close to the melting point of the carbides. It has appeared, however, in carrying on this method in practice that an undesirable coarsening of the grain of the material by crystalline transformation occurs due to the mass being heated up too close to the melting point, not to speak of the required high temperatures which are difficult to govern but have to be observed rather exactly. Therefore, the use of sintered pure carbides and carbide mixtures has been wholly given up in practice and the strength of the sintered shaped bodies has been improved by addition of more easily melting metals, so-called auxiliary metals, whereby simultaneously the sinter temperature could be notably lowered. So, for example, the sinter temperature of a mixture of tungsten carbide and 5% cobalt is about 1450° C. and thus is many hundred degrees lower than the sinter temperature of tungsten carbide not containing such auxiliary addition.

The addition of such auxiliary metals, however, prevents full utilization of the hardness of tungsten carbide so that the resistance to wear of these carbides is not so high as that of carbides not containing auxiliary metal. Therefore one has looked out for ways how the high sinter temperatures required for pure carbides could be reduced, with simultaneous increase of the strength of the shaped bodies. One of these ways, for example, consists in heating such carbides not containing auxiliary metal with simultaneous application of pressure, in order to obtain reduction of the sinter temperature. Furthermore, it has been proposed to favor the sinter effect by the action of high frequency currents during the application of pressure. These methods, however, are compara-

tively complicated and, moreover, it is difficult to produce under these conditions tool bodies of any desired configuration.

Therefore our invention has for its object to produce carbides of metals of high melting point showing great hardness and also strength, without any addition of auxiliary metal and at temperatures far remaining below the melting point of the carbides, and, finally, without simultaneous application of mechanical pressure. As stated by exhaustive tests, this object is achieved according to the invention by a proper selection of several carbides of metals of high melting point, viz, by admixing to a mixture of tungsten carbide and tantalum carbide one or several carbides of titanium, bolybdenum, vanadium, niobium, zirconium or thorium in a quantity of more than 5%, the mixture of tungsten carbide and tantalum carbide amounting to more than 50% of the alloy mass. Of the powdered mixture of these carbides, after having been shaped in the usual manner, can be prepared bodies of very great hardness and strength by sintering at 1400-1700° C. which bodies owing to their fine-grained texture show high cutting capacity and toughness. Best results are obtained if the quantity of the additional carbides amounts to from 10 to 20%.

The reason for a mixture prepared according to our invention sintering so dense at the comparatively low temperatures indicated might be due to the chemical transformations of the simultaneously present tungsten carbide and tantalum carbide with the additional other carbide or carbides, for, tungsten carbide or tantalum carbide alone or even a mixture of tungsten carbide and tantalum carbide require far higher sinter temperatures. The same is the case with the other carbides of metals of high melting point used besides tungsten carbide and tantalum carbide.

An hard alloy composed according to our invention and finished by sintering may have for example the following composition:

|                  | Parts by weight |    |
|------------------|-----------------|----|
| Tungsten carbide | 70              | 45 |
| Tantalum carbide | 15              |    |
| Titanium carbide | 15              |    |

The sinter temperature of this mixture lies at 1550° C. and thus is about the same as the sinter temperature of the commercial hard metals containing auxiliary metals, such as tungsten carbide containing an addition of cobalt, and this temperature is by many hundred degrees lower than the sinter temperature of a single carbide. 55

A further example may be the following carbide mixture:

|                    | Parts by weight |
|--------------------|-----------------|
| Tungsten carbide   | 50              |
| Molybdenum carbide | 10              |
| Tantalum carbide   | 30              |
| Vanadium carbide   | 10              |

The sinter temperature of this mixture lies at 1450° C., that is, it is likewise so low that a fine-grained texture is obtained as it is required to achieve favorable mechanical properties.

Practical tests of the hard alloys produced according to our invention have shown that the alloys are remarkable for an extraordinarily low wear, for example when used as drawing dies or in the cutting treatment, such as in turning grey cast iron or hard and soft steels, so that tools manufactured from these alloys are very economical in use.

What we claim and desire to secure by Letters Patent is:

1. The process of producing hard alloys consisting in preparing a powdered mixture of tungsten carbide and tantalum carbide, adding to this mixture at least one carbide of titanium, molybdenum, vanadium, niobium, zirconium or thorium in a quantity of more than 5%, the mixture of tungsten carbide and tantalum carbide amounting to more than 50% of the mass, pressing the mixture into shapes and sintering them at 1400°-1700° C.

2. The process of producing hard alloys consisting in preparing a powdered mixture of tungsten carbide and tantalum carbide, adding to this mixture at least one carbide of titanium, molybdenum, vanadium, niobium, zirconium or thorium in a quantity of from 10 to 20%, pressing the mixture into shapes and sintering them at 1400°-1700° C.

3. The process of producing a hard alloy, consisting in preparing a powdered mixture of 70 parts by weight tungsten carbide, 15 parts by weight tantalum carbide, and 15 parts by weight titanium carbide, pressing this mixture into shapes and sintering them at 1550° C.

4. The process of producing a hard alloy consisting in preparing a mixture of 50 parts by weight tungsten carbide, 30 parts by weight tantalum carbide, 10 parts by weight molybdenum carbide, and 10 parts by weight vanadium carbide, pressing the mixture into shapes and sintering them at 1450° C.

5. A sintered composition consisting of tungsten carbide and tantalum carbide and at least one carbide from the group consisting of titanium, molybdenum, vanadium, niobium, zirconium and thorium, the combined quantity of tungsten carbide and tantalum carbide being greater than 50% of said composition and the material from said group comprising more than 5% of said composition.

6. A sintered composition consisting of a mixture of tungsten carbide and tantalum carbide and at least one carbide from the group consisting of titanium, molybdenum, vanadium, niobium, zirconium and thorium, the metal from said group comprising 10 to 20% of said composition.

7. A sintered composition consisting of 70% tungsten carbide, 15% tantalum carbide and 15% titanium carbide.

8. A sintered composition consisting of 50% tungsten carbide, 30% tantalum carbide, 10% molybdenum carbide and 10% vanadium carbide.

WALTHER DAWIHL.  
KARL SCHRÖTER.